

## UNITED STATES PATENT OFFICE

2,439,281

FLASHLESS PROPELLANT POWDER  
COMPOSITIONGeorge Barsky, New York, N. Y., assignor to E. F.  
Drew & Co., Inc., a corporation of DelawareNo Drawing. Application March 7, 1942,  
Serial No. 433,717

7 Claims. (Cl. 52—5)

1

The present invention is directed to propellant powders, such as of the nitrocellulose type and more particularly, to compositions containing agents intended to assist in the formation of the nitrocellulose into granular form, and to reduce flash of the powder.

In converting nitrocellulose into powder grains it is customary to add certain substances, usually organic in nature, and sometimes having explosive properties in order to plasticize the nitrocellulose and render it more easily extruded or molded to the desired size and shape. However, most of the substances heretofore used for this purpose have but very limited solvent action on the nitrocellulose so that the plasticizing effect has been non-uniform, and the operation of incorporating the plasticizer has been quite slow. Even when heat is used in the process the operation is still slow and incomplete.

To overcome this it has been proposed to use various additions, as for example, certain ethers obtained from straight chain polyhydric alcohols, but such substances present further disadvantages. They are quite expensive to produce in that several chemical reactions are necessary and the operation is likely to result in by-products which are undesirable, and the efficiency of reaction thereby decreased.

It is also highly desirable in propellant powders to avoid a flash which normally occurs in a gun barrel when the gun is fired. Various substances have been added to the powder in an attempt to overcome this deficiency. However, various disadvantages are inherent in the substances previously used. Generally, a substance which reduces the flash of the powder is likely to produce a considerable amount of smoke. Among such substances are the dialkylphthalates which, while having the property of reducing the flash, give an excessive amount of black smoke when used in sufficient quantities to eliminate the flash. Also, other substances previously proposed for the purpose, have the disadvantage that they are more or less water-soluble and therefore increase the tendency of the powder to absorb moisture from the air.

The present invention is intended to provide a plasticizing agent for explosives such as of the nitrocellulose type wherein the plasticizer is simple in character, may be easily produced, and the raw materials for which are readily available.

It is also among the objects of the present invention to provide a propellant powder composition which shall be adapted to reduce the flash

2

resulting from ignition of the powder and at the same time not to adversely effect the moisture resistance of the powder.

The present invention also contemplates a plasticizer and a plasticized composition in which there is a high degree of solvent power for the nitrocellulose and in which there is a sufficient amount of lubrication by the plasticizer to render the extrusion of the nitrocellulose simple and rapid.

In practicing the present invention I provide an agent which consists essentially of an ester of a lower fatty acid having from 6 to 14 carbon atoms. Preferably acids from 8 to 12 carbon atoms are used, such as caprylic, capric and lauric acids. Acids of this type are esterified by means of a glycol ether or polyglycol. Usually the di- and tri-ethylene and propylene glycols are used. The esterification of the acid with the glycol may be conducted as is well-known, since the reaction follows the well-known esterification procedure.

The agent may be added to the explosive material or composition in relatively small amount to exert its solvent and lubricating effects. The following is an example of the character of the compositions which have been found useful:

|                                                                                                                                                                                                                                                                                    | Parts by weight |
|------------------------------------------------------------------------------------------------------------------------------------------------------------------------------------------------------------------------------------------------------------------------------------|-----------------|
| Nitrocellulose                                                                                                                                                                                                                                                                     | 30              |
| Tri-ethylene glycol caprylate                                                                                                                                                                                                                                                      | 1               |
|                                                                                                                                                                                                                                                                                    |                 |
| 30                                                                                                                                                                                                                                                                                 |                 |
| The amount of the agent may be varied to a considerable extent, depending upon the character of the nitrocellulose, the size of the grain to be produced, the nature of modifying ingredients, if any, the speed with which extrusion is to take place, and various other factors. |                 |

It has been found that a mixed ester is eminently suitable for the purpose. This is formed by first providing a composition of the following character:

|               | Parts by weight |
|---------------|-----------------|
| Caprylic acid | 8               |
| Capric acid   | 1               |

The mixture of acids is fully esterified with di- or tri-ethylene glycol in the well-known manner. It is believed that the reaction results in the formation of mixed esters as well as a mixture of simple esters. Such a composition has excellent solvent power for nitrocellulose and the like, and in addition, is capable of imparting a high degree of lubrication to the resultant mixture even in compositions where the mixed ester is used in quite small proportions. A mixture of nitrocellulose and the aforesaid composition, usually with the addition of a suitable amount of

volatile solvent in accordance with well-established practice, may be rapidly extruded through suitable dies with the formation of threads of smokeless powder. The threads, either before or after evaporation of the volatile solvent, can be cut into suitable lengths to give grains of desired size and shape. Compositions of this character may also be molded to produce the desired shape of bodies of the smokeless powder.

The new plasticizing material is eminently suitable for use in flashless powders. An example of such composition is as follows:

|                                             | Parts by weight |
|---------------------------------------------|-----------------|
| Nitrocellulose                              | 85              |
| Dinitrotoluol                               | 10              |
| Mixed tri-ethylene glycol caprylate-caprate | 5               |

The addition of the new plasticizer imparts excellent plasticity for the extrusion. Furthermore, the ester does not give off any material amount of smoke when burned and is flashless when incorporated in military powders. This is in direct contrast to the smokiness generated upon the burning of such plasticizers as the di-alkyl phthalates, for instance, di-butyl phthalate.

Another composition of similar nature which will provide a flashless propellant is as follows.

|                            | Parts by weight |
|----------------------------|-----------------|
| Nitrocellulose             | 80              |
| Trinitrotoluol             | 15              |
| Propylene glycol caprylate | 5               |

It is believed that the fact that the agents of the present invention have an oily nature, contributes largely to the effectiveness thereof in the extrusion operation, since such oily products give excellent lubricating effects. The plasticizers act rapidly as colloidizing agents and thus insure a uniform composition of the finished explosives. Furthermore, the agents are non-hygroscopic and therefore impart such properties to the explosive whereby the tendency to absorb moisture from the air is to a great extent eliminated. It is believed that the aliphatic nature of the plasticizer is responsible for the maintenance of the flashless character of the powder. All these factors result in a superior finished product.

Compositions made in accordance with the present invention may be used with or without the addition of other ingredients thereto. For instance, it is common to add to smokeless powders, a stabilizer such as diphenylamine, and additions of this character may be made to the present compositions without adversely effecting the same.

The proportions of the ingredients may be varied within wide limits, depending on the character of the explosive and other factors including the type of gun in which the explosive is to be used. The plasticizer may range from 2 to 10% of the mixture and the dinitrotoluol may be as much as 15% or more. Other mixtures than the above may be treated as set forth herein, and in such cases, the amount of plasticizer will vary in accordance with the solvent power thereof for the explosive material or composition and other properties.

The above examples are intended to be illus-

trative of the invention and do not limit the same, the scope of the invention being set forth in the claims appended hereto.

What is claimed is:

5 1. A propellant powder comprising an explosive consisting essentially of nitrocellulose having incorporated therein a minor amount of a composition which is the substantially neutral ester of a glycol taken from the class consisting of ethylene and propylene glycols with an acid taken from the class consisting of caprylic, capric and lauric acids.

10 2. A propellant powder comprising an explosive consisting essentially of nitrocellulose, having incorporated therein a minor amount of a composition which is the substantially neutral esters of diethylene glycol with an acid taken from the class consisting of caprylic, capric and lauric acids.

15 3. A propellant powder comprising an explosive which is a mixture of about 8 parts of a nitrocellulose and about 1 part of a nitrotoluol, having incorporated therein a minor amount of a composition which is the substantially neutral ester of a glycol taken from the class consisting of ethylene and propylene glycols with an acid taken from the class consisting of caprylic, capric and lauric acids.

20 4. A propellant powder comprising a nitrocellulose explosive having incorporated therein a minor amount of a composition which is the substantially neutral mixed esters of triethylene glycol with a mixture of caprylic and capric acids.

25 5. A propellant powder comprising a nitrocellulose explosive and a minor amount of the mixed poly-ethylene glycol esters of caprylic and capric acids, the caprylic being greater in amount than the capric acid.

30 6. A propellant powder comprising a nitrocellulose explosive and a minor amount of the mixed poly-ethylene glycol esters of caprylic and capric acids, the ratio of caprylic to capric acid being about 8 to 1.

35 7. A propellant powder comprising an explosive consisting essentially of nitrocellulose, having incorporated therein a minor amount of a composition which is the substantially neutral ester of triethylene glycol with an acid taken from the class consisting of caprylic, capric and lauric acids.

GEORGE BARSKY.

#### REFERENCES CITED

The following references are of record in the file of this patent:

#### UNITED STATES PATENTS

| Number    | Name     | Date          |
|-----------|----------|---------------|
| 2,031,603 | Holt     | Feb. 25, 1936 |
| 2,076,772 | Goodyear | Apr. 13, 1937 |
| 2,115,716 | Hansen   | May 3, 1938   |
| 2,118,506 | Graves   | May 24, 1938  |
| 2,198,746 | Spurlin  | Apr. 30, 1940 |
| 2,221,674 | Ellis    | Nov. 12, 1940 |
| 2,229,226 | Reid     | Jan. 21, 1941 |
| 2,396,074 | Barsky   | Mar. 5, 1946  |

#### FOREIGN PATENTS

| Number  | Country       | Date          |
|---------|---------------|---------------|
| 356,256 | Great Britain | Sept. 7, 1931 |